

## UNITED STATES PATENT OFFICE

2,045,347

## PRODUCTION OF THREADS AND THE LIKE

Henry Dreyfus, London, England

No Drawing. Application October 17, 1932, Serial  
No. 638,177. In Great Britain November 2,  
1931

12 Claims. (Cl. 18—54)

This invention relates to the manufacture of artificial filaments, threads, yarns, ribbons, films and like spun products from solutions of organic esters of cellulose and especially cellulose acetate. In British Patent No. 356,170 processes are described for the manufacture of filaments and other spun products from solutions of cellulose esters of low degree of esterification i. e. esters having less than two ester groups per cellulose molecule  $C_6H_{10}O_5$ . The said patent refers to dissolving the said esters in mixtures of acetone with water for the purpose of manufacturing the spun products. I have now found that improved results may be obtained by employing as solvent for esters of low ester content, e. g. those described in the above-mentioned patent, mixtures of acetone or like ketone, which is a solvent for the more highly esterified cellulose, with alcohols, and especially methyl and ethyl alcohols, with or without water.

The proportion of acetone to alcohol may vary considerably and is to some extent dependent upon the ester content of the cellulose ester. The alcohol may, for example, constitute as much as 50% of the total solvent mixture with cellulose diacetates or cellulose acetates of slightly lower acetyl content. Usually good results are obtainable with proportions of 30—40% of alcohol and 70—60% of acetone. With an acetate of 52% acetyl content, somewhat less alcohol may be used. The alcohol in the above mixtures may be partly replaced by water. For example, with a cellulose acetate having an acetyl value of about 48% a solvent mixture may comprise 60—75% of acetone 20—35% of methyl or ethyl alcohol and 5—10% of water. Instead of acetone other ketones may be used as for example methyl ethyl ketone.

Cellulose esters of relatively low ester content for use in this invention may be prepared by any suitable process. Thus for example they may be prepared by the hydrolysis (ripening) or saponification of cellulose esters of relatively high ester content.

Not only are the advantages, and notably the improved moisture regain, exhibited by the filaments, threads and the like of British specification No. 356,170 also attained in the process according to the present invention but in addition, inasmuch as it is possible to replace far more acetone by alcohol or by mixtures of alcohol and water than is possible in the case of water only, considerable economies can be effected. Moreover, I find that when spinning at high speed, for example 200—300 metres per minute or more, the residual solvent mixture left in the filaments

may be of such low solvent power that its subsequent action on the filaments or other products does not materially decrease their covering power. When employing acetone alone or acetone mixed with relatively small quantities of water, this phenomenon may detract somewhat from the commercial value of the products.

The above spinning solutions may be spun by dry or wet spinning methods. The spinning conditions will, of course, be adjusted in accordance with the nature of the product desired. For example the spinning conditions may be adjusted so as to obtain filaments of round cross-section or of relatively flat cross-section, or they may be adjusted to obtain hollow or voluminous filaments, it being generally desirable, in the case of dry spinning, to increase the spinning temperature in the neighbourhood of the spinning nozzles and/or to increase the rate of flow of the evaporative medium or the temperature of the spinning solution immediately prior to extrusion to achieve this latter result. In dry spinning operations, the temperatures necessary to obtain a particular result, employing as solvent mixture the mixture characteristic of the invention, are in general somewhat higher than those which may be used to obtain similar products using acetone or mixtures of acetone with small quantities of water.

Filaments prepared from the spinning solutions described herein may be stretched in any suitable manner, or may be shrunk, if desired, by any suitable process. Such filaments may also be submitted to partial or total saponification, or treated by processes calculated to modify their dyeing properties. Processes according to the present invention may also be used in conjunction with processes for reducing or modifying the lustre of the filaments.

The following example will serve to illustrate the invention, but it is not to be considered as limiting it in any way.

*Example*

Cellulose acetate of acetyl content 48% (calculated as acetic acid) obtained by hydrolysis of a cellulose acetate of higher acetyl value is dissolved to form a 25% solution in a solvent mixture consisting of 70 parts of acetone, 25 parts of ethyl alcohol and 5 parts of water. The solution so obtained is extruded from suitable orifices into a heated evaporative medium such as air or other gas maintained for example at a temperature of 75—85° C. and the filaments thus formed are associated by twisting.

The invention is particularly important in re-

lation to the spinning of filaments and like products from cellulose acetates, but may also be employed for the production of filaments and other products from cellulose propionates, cellulose butyrates, cellulose formates, cellulose nitroacetates and like organic esters of cellulose and mixed ether-esters of cellulose such as ethyl cellulose acetate and oxyethyl cellulose acetate.

What I claim and desire to secure by Letters Patent is:—

- 10 1. In a process for the production of artificial filaments, yarns, bristles, straw, ribbons and the like, which comprises spinning into a setting medium a solution containing as sole cellulose ester an organic ester of cellulose of relatively low degree of esterification, the step of forming said solution by dissolving said organic ester of cellulose in a solvent mixture containing a substance selected from the group consisting of acetone and methyl ethyl ketone, and an alcohol.
- 15 2. In a process for the production of artificial filaments, yarns, bristles, straw, ribbons and the like, which comprises spinning into a setting medium a solution containing as sole cellulose ester an organic ester of cellulose containing less than two ester radicles per molecule of cellulose considered as  $C_6H_{10}O_5$ , the step of forming said solution by dissolving said organic ester of cellulose in a solvent mixture containing acetone and a lower fatty alcohol.
- 20 3. In a process for the production of artificial filaments, yarns, bristles, straw, ribbons and the like, which comprises spinning into an evaporative atmosphere a solution containing as sole cellulose ester cellulose acetate containing less than two acetate radicles per molecule of cellulose considered as  $C_6H_{10}O_5$ , the step of forming said solution by dissolving said cellulose acetate in a solvent mixture containing acetone and methyl alcohol.
- 25 4. Process according to claim 3 wherein a cellulose acetate having an acetyl value of at least 40%, calculated as acetic acid, is employed.
- 30 5. Process according to claim 3 wherein a cellulose acetate having an acetyl value of at least 45%, calculated as acetic acid, is employed.
- 35 6. In a process for the production of artificial filaments, yarns, bristles, straw, ribbons and the like, which comprises spinning into an evaporative atmosphere a solution containing as sole cellulose ester cellulose acetate containing less than two acetate radicles per molecule of cellulose considered as  $C_6H_{10}O_5$ , the step of forming said solution by dissolving said cellulose acetate in a solvent mixture containing acetone and ethyl alcohol.

7. In a process for the production of artificial filaments, yarns, bristles, straw, ribbons and the like, which comprises spinning into an evaporative atmosphere a solution containing as sole cellulose ester cellulose acetate containing less than two acetate radicles per molecule of cellulose considered as  $C_6H_{10}O_5$ , the step of forming said solution by dissolving said cellulose acetate in a solvent mixture containing acetone, water and methyl alcohol.

8. In a process for the production of artificial filaments, yarns, bristles, straw, ribbons and the like, which comprises spinning into an evaporative atmosphere a solution containing as sole cellulose ester cellulose acetate containing less than two acetate radicles per molecule of cellulose considered as  $C_6H_{10}O_5$ , the step of forming said solution by dissolving said cellulose acetate in a solvent mixture containing acetone, water and ethyl alcohol.

9. In a process for the production of artificial filaments, yarns, bristles, straw, ribbons and the like, which comprises spinning into a setting medium a solution containing as sole cellulose ester an organic ester of cellulose having an acyl content below the minimum necessary for solubility in pure acetone, the step of forming said solution by dissolving said organic ester of cellulose in a solvent mixture containing acetone and a lower fatty alcohol.

10. In a process for the production of artificial filaments, yarns, bristles, straw, ribbons and the like, which comprises spinning into an evaporative atmosphere a solution containing as sole cellulose ester cellulose acetate having an acetyl content below the minimum necessary for solubility in pure acetone, the step of forming said solution by dissolving said cellulose acetate in a solvent mixture containing acetone and ethyl alcohol.

11. A spinning solution for the production of filaments, yarns, bristles, straw, ribbons, films and the like comprising an organic ester of cellulose of relatively low ester content dissolved in a solvent medium containing acetone and a lower fatty alcohol, said ester being the only cellulose ester present in the solution.

12. A spinning solution for the production of filaments, yarns, bristles, straw, ribbons and the like, which comprises a cellulose acetate containing less than two acetyl radicles per molecule of cellulose, considered as  $C_6H_{10}O_5$ , dissolved in a solvent mixture comprising acetone and ethyl alcohol, said cellulose acetate being the only cellulose ester present in the solution.

HENRY DREYFUS.